

1

3,112,207  
FLUOALUMINATE COMPOSITION AS  
DIELECTRIC MATERIAL

Isadore Mockrin, Plymouth Meeting, and Alexander Kowalski, Levittown, Pa., assignors to Pennsalt Chemicals Corporation, Philadelphia, Pa., a corporation of Pennsylvania  
No Drawing. Filed Oct. 11, 1961, Ser. No. 144,308  
6 Claims. (Cl. 106—39)

This invention relates to a novel composition comprised of certain fluoaluminates and their use as novel dielectric materials. More particularly, the invention deals with solid solutions consisting essentially of potassium tetrafluooaluminate, rubidium tetrafluooaluminate and potassium fluoborate and the use of such solid solutions as dielectric materials.

A dielectric or insulating material may be characterized roughly as having an electrical conductivity less than  $10^{-6}$  mhos/cm. Important dielectrics include mica, barium titanate, various ceramics, paper and impregnated papers, numerous plastics and the like. Muscovite,



and phlogopite,  $K_4Mg_{12}Al_4Si_{12}O_{40}(OH)_8$  are the two natural forms of mica used as dielectrics. Synthetic mica, phlogopite in which F has replaced the OH group, is also used to some extent. Such characteristics as high dielectric strength, low power-factor losses, flexibility, transparency and perfect cleavage make mica usable in many industries.

Sheet mica is a vital material both in peace and wartime for the electronic and electrical industries. Unfortunately, the United States has been virtually dependent on foreign sources for high-quality sheet mica. India is the principal source of muscovite sheet mica. Brazil is also an important exporter of high-quality muscovite block to the United States, the United States' supply of phlogopite is obtained almost entirely from Madagascar and Canada.

Research on synthetic mica, or fluorine-phlogopite, has resulted in a commercially feasible method for manufacture, but only relatively small crystals are generally obtained, so that synthetic mica is not a substitute for sheet mica. However, synthetic mica is used in such applications as glass-bonded mica ceramics and hot-pressed machinable dielectrics (see for example, the disclosure of U.S. 2,675,853). Thus, there still remains the need for a readily available sheet dielectric material.

In the application of I. Mockrin, Serial No. 39,726, filed June 29, 1960, issued January 9, 1962, as U.S. 3,016,480, there is described the use of potassium or rubidium tetrafluooaluminates as dielectric materials. These fluoaluminates may be obtained in a layer structure form providing cleavable sheets similar to natural mica. It has been observed when working with potassium and rubidium tetrafluooaluminates that  $KAIF_4$  forms less brittle and larger crystalline sheets than does  $RbAlF_4$ . On the other hand,  $RbAlF_4$  forms "books" of crystals which cleave more readily than  $KAIF_4$ . Furthermore, it has been observed that at low temperatures (about  $-23^{\circ}C$ ),  $KAIF_4$  undergoes a transition which results in deterioration of the desirable sheet structure.

However, in application Serial No. 102,518, filed on April 12, 1961, by Isadore Mockrin and Alexander Kowalski, it is pointed out that the transition temperature can be greatly lowered and that improved cleavage properties

2

are obtained by providing a composition which is a solid solution of  $KAIF_4$  and  $RbAlF_4$ .

It has now been found by this invention that improved fluoaluminite dielectric materials are obtained by providing novel compositions which comprise solid solutions of  $KAIF_4$ ,  $RbAlF_4$  and  $KBF_4$ . Such novel compositions have the unexpected properties of large size crystals and good cleavability and they offer advantages from the standpoint of preparation and ease of fabrication.

10 The novel compositions of this invention include those mixtures of the ternary solid solution of  $KAIF_4$ ,  $RbAlF_4$  and  $KBF_4$  which contain about 1 to about 15 mol percent of  $KBF_4$  and at least about 4 mol percent of  $RbAlF_4$ . These levels of ingredients are significant because below about 4 mol percent of  $RbAlF_4$ , the transition temperature of the solid solution is not lowered to the desired level. Expressed another way, it requires at least about 4 mol percent of  $RbAlF_4$  in the ternary solid solution to achieve the low transition temperature advantages. The upper limit of  $RbAlF_4$  will be about 90 mol percent since a greater amount in the composition reduces crystal flexibility. A molar proportion of  $KBF_4$  in the range between about 1% and 5% is preferred in order to achieve optimum properties for the ternary solid solution. At levels of below about 1%, the amount of  $KBF_4$  does not add materially to improved cleavage properties. On the other hand, even when  $KBF_4$  is used in the melt in amounts exceeding about 15% the ternary product still contains only about 15% because this appears to be the solubility limit of  $KBF_4$  in the ternary composition. From a practical standpoint the ternary composition will preferably contain between about 4% and 50% rubidium tetrafluooaluminate and from about 2% to 5% of potassium fluoborate, the balance being the potassium tetrafluooaluminate.

35 The novel dielectric compositions of this invention are readily obtained by slowly cooling a melt of the three ingredients, no elaborate controls being required. In this way relatively large sheet-like crystals of the ternary solid solution formed. After cooling the melt, the resulting material contains "books" of sheet-like crystals of varying size which after removal are split and used in the manner normally employed with mica.

40 The potassium fluoborate ingredient of the ternary solid solution is a well known composition prepared from  $H_3BO_3$  and HF in the presence of potassium hydroxide according to the method of Borlander, Hollatz, and Fisher (Ber., vol. 65, page 535, 1932).

45 The fluoaluminite materials (e.g.  $KAIF_4$  and  $RbAlF_4$ ) are prepared readily according to the method of Brosset (Z. Anorg. Chem., 235, 139-147 (1937) and 239 301-304 (1938) which involves simply the evaporation to dryness of a mixture of (1) an aqueous hydrogen fluoride solution of a hydrated alumina (e.g. gibbsite), and (2) the alkali metal (i.e. potassium or rubidium) fluoride, the solid ingredients being used in stoichiometric amounts.

50 As indicated, these novel fluoaluminite compositions are solid solutions, by which is meant that the lattice structure of neither constituent is evident in X-ray patterns, but that a composite, single-phase lattice, intermediate between that of the three constituents is observed. The crystalline sheets of this solid solution are transparent, have excellent cleavage properties and in addition show no transition when cooled to temperatures below  $-78^{\circ}C$ . It is quite surprising that  $KBF_4$  exhibits solid solubility in admixture with  $KAIF_4$  and  $RbAlF_4$ . The crystal lattice structure of  $KAIF_4$  and  $RbAlF_4$  theoretically requires that any element substituting for aluminum in the lattice net-

work have a coordination number of 6. Boron has a coordination number of 3 or 4, but never 6 and yet it exhibits solid solubility in admixture with  $\text{KAlF}_4$  and  $\text{RbAlF}_4$ .

The following examples will serve to further illustrate the invention:

#### EXAMPLE 1

99.5 parts of potassium tetrafluoroaluminate, 131.9 parts of rubidium tetrafluoroaluminate, and 5.0 parts of potassium tetrafluoborate were fused at  $650^\circ\text{C}$ . for one hour and then cooled slowly until solid. The matrix contained many books of transparent sheet crystals, some of which were  $\frac{1}{2}$  inch by  $\frac{1}{2}$  inch. These sheets were cleaved readily to crystals less than one mil thick. The thin crystals were strong and somewhat flexible. The melt composition yielding this product corresponded on a molar basis to 48.6%  $\text{KAlF}_4$ , 48.6%  $\text{RbAlF}_4$  and 2.8%  $\text{KBF}_4$ .

#### EXAMPLE 2

Following the essential details of Example 1, a melt composition containing on a molar basis 76.5%  $\text{KbAlF}_4$ , 8.5%  $\text{RbAlF}_4$  and 15%  $\text{KBF}_4$  was cooled to yield books of transparent sheet crystals easily cleavable to strong, mica-like materials.

#### EXAMPLE 3

A product similar to that of Example 2 was obtained from a melt composition of 42.5%  $\text{KAlF}_4$ , 42.5%  $\text{RbAlF}_4$  and 15%  $\text{KBF}_4$ .

#### EXAMPLE 4.—THERMAL DATA FOR LOW-TEMPERATURE INVERSION

The low-temperature "inversion" was studied by differential thermal analysis (DTA). The furnace and sample holder for this low-temperature DTA consists of a Dewar flask thoroughly chilled with liquid nitrogen prior to the run and a silver sample block on which is wound a resistance winding of insulated wire connected to 110 v. A.C. with a variable voltage transformer. The rate of heating depends on the current applied (up to 1 amp.). Cooling curves were run and then heating curves. The former yielded exothermic peaks and the latter endothermic peaks; this is characteristic of inversions.

The following table illustrates the improvement obtained by this invention with respect to the low temperature inversion effect. It is clear from the table that the solid solutions of this invention show the transition at temperatures much below that for  $\text{KAlF}_4$  alone and are equivalent in this property to the low inversion temperatures obtained with the binary mixtures of S.N. 102,518 referred to above.

Table I

| Composition                         | Temperature of Transition on Cooling |
|-------------------------------------|--------------------------------------|
| $\text{KAlF}_4$                     | -23° C.                              |
| $\text{KAlF}_4$ —99 mole percent    | -39° C.                              |
| $\text{RbAlF}_4$ —1 mole percent    |                                      |
| $\text{KAlF}_4$ —95 mole percent    | Below -78° C.                        |
| $\text{RbAlF}_4$ —5 mole percent    |                                      |
| $\text{KAlF}_4$ —48.6 mole percent  | Below -106° C.                       |
| $\text{RbAlF}_4$ —48.6 mole percent |                                      |
| $\text{KBF}_4$ —2.8 mole percent    |                                      |
| $\text{KAlF}_4$ —75.5 mole percent  | Below -78° C.                        |
| $\text{RbAlF}_4$ —8.5 mole percent  |                                      |
| $\text{KBF}_4$ —15.0 mole percent   | Below -78° C.                        |
| $\text{KAlF}_4$ —42.5 mole percent  |                                      |
| $\text{RbAlF}_4$ —42.5 mole percent | Below -196° C.                       |
| $\text{KBF}_4$ —15.0 mole percent   |                                      |

#### EXAMPLE 5

Crystals of various thickness from various molar ratios of  $\text{KBF}_4$ — $\text{KAlF}_4$ — $\text{RbAlF}_4$  solid solutions were used as the dielectric of a capacitor.

Dielectric measurements were made at  $25^\circ\text{C}$ . with a General Radio Capacitance Bridge, Model 716-C, for the

frequencies 100 c.p.s., 1 kc. and 10 kc. For measurement at 100 kc. and higher, a Boonton Q Meter was used.

The test sample was a capacitor consisting of two electrodes separated by a solid spacer which spacer was the fluoaluminate sheet. The capacitor was prepared either (a) by vacuum depositing gold or (b) by applying a silver paint to the opposite flat faces of the fluoaluminate sheet and drying at  $200^\circ\text{C}$ . for 30 minutes, thus leaving the silver metal as electrodes.

Dielectric strength values were determined on crystal pieces with noncoated or with silver coated samples. The sample in the former case was held between point contacts immersed in an oil bath. The rate of loading, in accordance with an ASTM standard, was step-wise at 500 volts/minute, 60 cycles until failure. Since the dielectric strength is expressed as volts/unit thickness, the determination of the thickness of the piece investigated is required.

A micrometer measurement of the thickness gives a value which does not reflect localized variations of thickness. Therefore, it was considered more meaningful to first conduct the experiment until failure and subsequently measure the thickness in the immediate vicinity of failure by optical methods. A microscope at a 230 magnification was used. The vertical adjustment of the focal point by a micrometer screw calibrated in microns permits the measurement of thickness in the vicinity of breakdown. The true thickness of the sample is then the linear distance between a focus on the upper and lower crystal surfaces multiplied by the index of refraction. The index of refraction of these materials was assumed to be about 1.4 which is representative of crystalline inorganic fluorine-containing materials.

Both the above methods have been utilized for thickness measurements; however, for the purposes of determination of dielectric strength, the latter optical method is deemed preferable. In general, the test procedures of ASTM designation D 150-54T were followed.

The data given in the following tables represent values obtained in the dielectric tests when using the more physically perfect samples, having a general absence of cracks, striations and other imperfections. Tables II to V give the capacitance (C), dielectric constant (K) and dissipation factor ( $\tan \delta \times 10^{-4}$ ) for samples of various thickness at various frequencies.

Table II

MELT COMPOSITION: 87%  $\text{KAlF}_4$ —10%  $\text{RbAlF}_4$ —3%  $\text{KBF}_4$

| Sample                                                                  | Frequency  | Tan $\delta \times 10^{-4}$ | C, $\mu\text{uf.}$ | K    |
|-------------------------------------------------------------------------|------------|-----------------------------|--------------------|------|
| $t=.015 \text{ mm.}$<br>$A=24.86 \text{ mm.}^2$<br>$K=.0682 \text{ C.}$ | 100 c.p.s. | 192.8                       | 111.2              | 7.57 |
|                                                                         | 1 kc.      | 70.3                        | 108.7              | 7.40 |
|                                                                         | 10 kc.     | 18.1                        | 108.3              | 7.37 |
|                                                                         | 1 mc.      | 65.70                       | 107.5              | 7.34 |
|                                                                         | 3 mc.      | 51.80                       | 82.25              | 7.14 |
|                                                                         |            | 101.7                       | 80.41              | 6.95 |
| $t=.055 \text{ mm.}$<br>$A=12.67 \text{ mm.}^2$<br>$K=.490 \text{ C.}$  | 100 c.p.s. | 89.5                        | 17.9               | 8.77 |
|                                                                         | 1 kc.      | 26.0                        | 17.7               | 8.68 |
|                                                                         | 10 kc.     | 9.7                         | 17.65              | 8.65 |
|                                                                         | 1 mc.      | 29.4                        | 17.20              | 8.43 |
|                                                                         | 3 mc.      | 40.5                        | 16.74              | 8.20 |
|                                                                         |            |                             |                    |      |
| $t=.02 \text{ mm.}$<br>$A=11.79 \text{ mm.}^2$<br>$K=.192 \text{ C.}$   | 100 c.p.s. | 154.3                       | 37.8               | 7.26 |
|                                                                         | 1 kc.      | 44.4                        | 37.4               | 7.18 |
|                                                                         | 10 kc.     | 20.4                        | 37.25              | 7.15 |
|                                                                         | 1 mc.      | 71.3                        | 35.92              | 6.89 |
|                                                                         | 3 mc.      | 95.6                        | 34.57              | 6.64 |
|                                                                         |            |                             |                    |      |
| $t=.032 \text{ mm.}$<br>$A=10.01 \text{ mm.}^2$<br>$K=.361 \text{ C.}$  | 100 c.p.s. | 150.0                       | 25.90              | 9.34 |
|                                                                         | 1 kc.      | 56.6                        | 25.40              | 9.15 |
|                                                                         | 10 kc.     | 21.2                        | 25.40              | 9.15 |
|                                                                         | 1 mc.      | 83.1                        | 24.70              | 8.92 |
|                                                                         | 3 mc.      | 112.2                       | 23.30              | 8.41 |
|                                                                         |            |                             |                    |      |
| $t=.08 \text{ mm.}$<br>$A=17.49 \text{ mm.}^2$<br>$K=.194 \text{ C.}$   | 100 c.p.s. | 138.6                       | 36.75              | 7.13 |
|                                                                         | 1 kc.      | 55.3                        | 36.15              | 7.01 |
|                                                                         | 10 kc.     | 16.65                       | 36.00              | 6.98 |
|                                                                         | 1 mc.      | 47.9                        | 34.90              | 6.77 |
|                                                                         | 3 mc.      | 65.9                        | 33.66              | 6.53 |
|                                                                         |            |                             |                    |      |

LEGEND:

t=thickness of sample.  
A=area of one crystal face.  
K=dielectric constant.

5  
Table IIIMELT COMPOSITION: 77% KAlF<sub>4</sub>—20% RbAlF<sub>4</sub>—3% KBF<sub>4</sub>

| Sample                   | Frequency  | Tan $\delta \times 10^{-4}$ | C, $\mu\text{f}$ | K     | 5  |
|--------------------------|------------|-----------------------------|------------------|-------|----|
| t=.05 mm.                | 100 c.p.s. | 55.5                        | 43.2             | 10.70 |    |
| A=22.75 mm. <sup>2</sup> | 1 kc.      | 29.9                        | 42.8             | 10.62 |    |
| K=.248 C.                | 10 kc.     | 15.5                        | 42.6             | 10.57 |    |
|                          | 1 mc.      | 63.7                        | 42.7             | 10.60 |    |
|                          | 3 mc.      | 106.5                       | 39.9             | 9.90  |    |
| t=.045 mm.               | 100 eps.   | 31.1                        | 23.75            | 8.83  | 10 |
| A=13.64 mm. <sup>2</sup> | 1 kc.      | 12.8                        | 23.45            | 8.72  |    |
| K=372 C.                 | 10 kc.     | 8.6                         | 23.35            | 8.68  |    |
|                          | 1 mc.      | 32.5                        | 22.90            | 8.52  |    |
|                          | 3 mc.      | 60.4                        | 21.30            | 7.92  |    |

Legend:  
t=thickness of sample.  
A=area of one crystal face.  
K=dielectric constant.

15

Table IV

MELT COMPOSITION: 67% KAlF<sub>4</sub>—30% RbAlF<sub>4</sub>—3% KBF<sub>4</sub>

| Sample                   | Frequency  | Tan $\delta \times 10^{-4}$ | C, $\mu\text{f}$ | K    | 20 |
|--------------------------|------------|-----------------------------|------------------|------|----|
| t=.088 mm.               | 100 c.p.s. | 53.7                        | 11.15            | 8.13 |    |
| A=13.61 mm. <sup>2</sup> | 1 kc.      | 21.6                        | 11.10            | 8.11 |    |
| K=.731 C.                | 10 kc.     | 18.0                        | 11.10            | 8.11 |    |
|                          | 1 mc.      | 21.2                        | 10.56            | 7.72 | 25 |
|                          | 3 mc.      | 7.14                        | 10.92            | 8.00 |    |
| t=.065 mm.               | 100 c.p.s. | 22.5                        | 30.80            | 7.52 |    |
| A=30.12 mm. <sup>2</sup> | 1 kc.      | 13.1                        | 30.70            | 7.49 |    |
| K=.244 C.                | 10 kc.     | 11.7                        | 30.65            | 7.48 |    |
|                          | 1 mc.      | 14.4                        | 30.41            | 7.42 |    |
|                          | 3 mc.      | 9.85                        | 28.86            | 7.06 | 30 |
| t=.068 mm.               | 100 c.p.s. | 11.60                       | 89.60            | 7.19 |    |
| A=84.72 mm. <sup>2</sup> | 1 kc.      | 6.02                        | 89.50            | 7.18 |    |
| K=.0803 C.               | 10 kc.     | 4.69                        | 89.45            | 7.17 |    |
|                          | 1 mc.      | 10.46                       | 89.78            | 7.21 |    |
|                          | 3 mc.      | 13.80                       | 87.52            | 7.07 |    |
| t=.1 mm.                 | 100 c.p.s. | 8.25                        | 36.3             | 6.98 | 35 |
| A=58.72 mm. <sup>2</sup> | 1 kc.      | 5.50                        | 36.3             | 6.98 |    |
| K=.192 C.                | 10 kc.     | 2.75                        | 36.3             | 6.98 |    |
|                          | 1 mc.      | 10.52                       | 35.45            | 6.80 |    |
|                          | 3 mc.      | 16.40                       | 33.74            | 6.48 |    |
| t=.035 mm.               | 100 c.p.s. | 16.30                       | 43.00            | 7.34 |    |
| A=23.05 mm. <sup>2</sup> | 1 kc.      | 9.70                        | 42.95            | 7.36 | 40 |
| K=.1717 C.               | 10 kc.     | 6.5                         | 42.80            | 7.35 |    |
|                          | 1 mc.      | 33.4                        | 42.88            | 7.36 |    |
|                          | 3 mc.      | 51.4                        | 40.89            | 7.19 |    |

Legend:  
t=thickness of sample.  
A=area of one crystal face.  
K=dielectric constant.

10

6  
Table VI.—Dielectric StrengthMELT COMPOSITION: 87% KAlF<sub>4</sub>—10% RbAlF<sub>4</sub>—3% KBF<sub>4</sub>

| Thickness, <sup>1</sup> inches $\times 10^{-3}$ | Total Volts, 60 c.p.s. | Dielectric Strength, volts/mil |
|-------------------------------------------------|------------------------|--------------------------------|
| 2.36                                            | 8,000                  | 3,390                          |
| 2.50                                            | 6,500                  | 2,560                          |
| 2.08                                            | 5,500                  | 2,640                          |
| 2.11                                            | 7,000                  | 3,320                          |
| 1.75                                            | 4,000                  | 2,280                          |
| 1.98                                            | 6,000                  | 3,030                          |
| 2.26                                            | 8,500                  | 3,760                          |
| 2.59                                            | 6,000                  | 2,320                          |
| 1.62                                            | 6,500                  | 4,010                          |
| 3.52                                            | 8,000                  | 2,270                          |
| 3.99                                            | 6,500                  | 1,630                          |
| 2.54                                            | 4,500                  | 1,770                          |
| 2.55                                            | 4,500                  | 1,765                          |
| 1.39                                            | 3,000                  | 2,150                          |
| 1.60                                            | 6,500                  | 4,060                          |
| <sup>2</sup> 2.32                               | -----                  | <sup>2</sup> 2,730             |

<sup>1</sup> Measured optically [n=1.40 (assumed)].<sup>2</sup> Average values.

Table VII.—Dielectric Strength

MELT COMPOSITION: 77% KAlF<sub>4</sub>—20% RbAlF<sub>4</sub>—3% KBF<sub>4</sub>

| Thickness, <sup>1</sup> inches $\times 10^{-3}$ | Total Volts, 60 c.p.s. | Dielectric Strength, volts/mil |
|-------------------------------------------------|------------------------|--------------------------------|
| 1.54                                            | 2,500                  | 1,622                          |
| 1.65                                            | 3,500                  | 2,120                          |
| 2.56                                            | 6,500                  | 2,540                          |
| 1.56                                            | 2,500                  | 1,600                          |
| 1.72                                            | 3,500                  | 2,035                          |
| 1.96                                            | 5,000                  | 2,550                          |
| 2.89                                            | 7,000                  | 2,420                          |
| 2.63                                            | 6,000                  | 2,280                          |
| 2.53                                            | 7,500                  | 2,980                          |
| 2.86                                            | 8,000                  | 2,795                          |
| 3.03                                            | 8,000                  | 2,640                          |
| 2.56                                            | 7,000                  | 2,735                          |
| 2.37                                            | 5,000                  | 2,110                          |
| 2.04                                            | 3,500                  | 1,715                          |
| <sup>2</sup> 2.28                               | -----                  | <sup>2</sup> 2,290             |

<sup>1</sup> Measured optically [n=1.40 (assumed)].<sup>2</sup> Average values.

Table V

MELT COMPOSITION: 57% KAlF<sub>4</sub>—40% RbAlF<sub>4</sub>—3% KBF<sub>4</sub>

| Sample                   | Frequency  | Tan $\delta \times 10^{-4}$ | C, $\mu\text{f}$ | K     | 50 |
|--------------------------|------------|-----------------------------|------------------|-------|----|
| t=.05 mm.                | 100 c.p.s. | 5250                        | 61.60            | 10.70 |    |
| A=32.48 mm. <sup>2</sup> | 1 kc.      | 618                         | 55.20            | 9.58  |    |
| K=.174 C.                | 10 kc.     | 76.1                        | 54.90            | 9.54  |    |
|                          | 1 mc.      | 30.5                        | 54.10            | 9.42  |    |
|                          | 3 mc.      | 52.4                        | 52.30            | 9.18  |    |
| t=.047 mm.               | 100 c.p.s. | 21.20                       | 19.95            | 8.62  |    |
| A=12.01 mm. <sup>2</sup> | 1 kc.      | 6.05                        | 19.85            | 8.59  |    |
| K=.432 C.                | 10 kc.     | 6.02                        | 19.95            | 8.62  |    |
|                          | 1 mc.      | 46.20                       | 19.24            | 8.32  |    |
|                          | 3 mc.      | 59.50                       | 18.07            | 7.81  | 60 |
| t=.05 mm.                | 100 c.p.s. | 153                         | 40.40            | 7.47  |    |
| A=30.5 mm. <sup>2</sup>  | 1 kc.      | 39.0                        | 40.00            | 7.40  |    |
| K=.185 C.                | 10 kc.     | 21.1                        | 39.75            | 7.35  |    |
|                          | 1 mc.      | 26.8                        | 37.65            | 6.96  |    |
|                          | 3 mc.      | 40.6                        | 36.35            | 6.73  |    |
| t=.042 mm.               | 100 c.p.s. | 13.8                        | 36.35            | 9.45  | 65 |
| A=78.26 mm. <sup>2</sup> | 1 kc.      | 9.3                         | 36.30            | 9.44  |    |
| K=.260 C.                | 10 kc.     | 8.2                         | 36.25            | 9.43  |    |
|                          | 1 mc.      | 25.3                        | 34.98            | 9.10  |    |
|                          | 3 mc.      | 59.4                        | 33.79            | 8.78  |    |

Legend:

t=thickness of sample.  
A=area of one crystal face.  
K=dielectric constant.

45

Table VIII.—Dielectric Strength

MELT COMPOSITION: 67% KAlF<sub>4</sub>—30% RbAlF<sub>4</sub>—3% KBF<sub>4</sub>

| Thickness, <sup>1</sup> inches $\times 10^{-3}$ | Total Volts, 60 c.p.s. | Dielectric Strength, volts/mil |
|-------------------------------------------------|------------------------|--------------------------------|
| 1.57                                            | 6,500                  | 4,140                          |
| 1.98                                            | 7,000                  | 3,530                          |
| 1.97                                            | 6,500                  | 3,300                          |
| 2.65                                            | 4,500                  | 1,700                          |
| 1.76                                            | 5,000                  | 2,840                          |
| 1.72                                            | 5,000                  | 2,910                          |
| 2.23                                            | 5,500                  | 2,470                          |
| 2.48                                            | 6,500                  | 2,620                          |
| 1.57                                            | 5,000                  | 3,180                          |
| 1.01                                            | 4,000                  | 3,980                          |
| 2.58                                            | 6,000                  | 2,320                          |
| 2.42                                            | 8,000                  | 3,310                          |
| 2.05                                            | 7,500                  | 3,660                          |
| 2.46                                            | 7,500                  | 3,045                          |
| 2.60                                            | 4,000                  | 1,540                          |
| <sup>2</sup> 2.07                               | -----                  | <sup>2</sup> 2,970             |

<sup>1</sup> Measured optically [n=1.40 (assumed)].<sup>2</sup> Average values.

The following Tables VI and IX illustrate the dielectric strength properties of the compositions of the invention and Table X is for comparative value with muscovite mica. 75

7  
*Table IX.—Dielectric Strength*MELT COMPOSITION: 57%  $\text{KAlF}_4$ —40%  $\text{RbAlF}_4$ —3%  $\text{KBF}_4$ 

| Thickness, <sup>1</sup><br>inches $\times 10^{-3}$ | Total Volts,<br>60 c.p.s. | Dielectric<br>Strength,<br>volts/mil |
|----------------------------------------------------|---------------------------|--------------------------------------|
| 1.65                                               | 5,500                     | 3,330                                |
| 1.78                                               | 5,000                     | 2,810                                |
| .75                                                | 4,500                     | 5,975                                |
| 1.46                                               | 4,000                     | 2,740                                |
| 1.08                                               | 3,500                     | 3,240                                |
| 1.27                                               | 2,500                     | 1,970                                |
| 1.87                                               | 8,500                     | 4,540                                |
| 2.20                                               | 9,000                     | 4,080                                |
| 1.57                                               | 6,500                     | 4,140                                |
| 2.02                                               | 6,000                     | 2,970                                |
| 1.28                                               | 3,500                     | 2,740                                |
| 1.56                                               | 7,000                     | 4,480                                |
| 1.60                                               | 4,500                     | 2,810                                |
| 1.75                                               | 7,500                     | 4,280                                |
| 3.10                                               | 5,500                     | 1,775                                |
| <sup>2</sup> 1.66                                  |                           | <sup>2</sup> 3,460                   |

<sup>1</sup> Measured optically [ $n=1.40$  (assumed)].<sup>2</sup> Average values.

For comparative purposes Table X is included to show the dielectric strength properties of a commercial mica.

8  
*Table X*

COMPOSITION: COMMERCIAL MUSCOVITE MICA

| Sample | Thickness, <sup>1</sup><br>inches<br>$\times 10^{-3}$ | Total Volts,<br>60 c.p.s. | Dielectric<br>Strength,<br>volts/mil |
|--------|-------------------------------------------------------|---------------------------|--------------------------------------|
| 1      | 1.16                                                  | 4,500                     | 3,880                                |
| 2      | 1.99                                                  | 8,500                     | 4,270                                |
| 3      | 1.74                                                  | 6,500                     | 3,730                                |
| 4      | 1.19                                                  | 3,000                     | 2,520                                |
| 5      | 0.875                                                 | 3,500                     | 4,000                                |
| 6      | 2.38                                                  | 9,000                     | 3,780                                |
| 7      | 2.58                                                  | 9,000                     | 3,490                                |
| 8      | 2.78                                                  | 9,500                     | 3,420                                |
| 9      | 3.04                                                  | 6,500                     | 2,140                                |
| 10     | 2.69                                                  | 5,500                     | 2,040                                |
| 11     | 1.66                                                  | 7,500                     | 4,520                                |
| 12     | 3.30                                                  | 9,500                     | 2,880                                |
| 13     | 0.70                                                  | 4,000                     | 5,680                                |
| 14     | 0.67                                                  | 3,500                     | 5,220                                |
| 15     | 0.86                                                  | 4,000                     | 4,650                                |

<sup>1</sup> Measured optically [ $n=1.59$  (mean value for muscovite)].

It is clear that the dielectric strength properties of the compositions of this invention have the same order of magnitude as the commercial mica. It will be evident from the above data that the dielectric strength properties do not appear to vary with the composition of the solid solutions of this invention. However, there does appear to be a tendency toward the same thickness effect reported with muscovite mica in that the greatest dielectric strength is obtained with the thinnest samples. This invention provides for compositions with good cleaving properties and thus enables thin crystal sheets to be readily obtained resulting in dielectric materials of relatively high dielectric strength.

## EXAMPLE 6

Observations concerning the effect of composition on ease of cleaving of the crystals are listed in Table XI:

Table XI

OBSERVATIONS CONCERNING THE CLEAVABILITY OF  $\text{KAlF}_4$  AND  $\text{KAlF}_4$ — $\text{RbAlF}_4$ — $\text{KBF}_4$  CRYSTALS

| 5  | Composition, mol percent                                         | Remarks                                                                       |
|----|------------------------------------------------------------------|-------------------------------------------------------------------------------|
|    | 100% $\text{KAlF}_4$                                             | Hard to cleave—Brittle layers not continuous.                                 |
| 10 | 87% $\text{KAlF}_4$<br>10% $\text{RbAlF}_4$<br>3% $\text{KBF}_4$ | Readily cleavable.                                                            |
|    | 77% $\text{KAlF}_4$<br>20% $\text{RbAlF}_4$<br>3% $\text{KBF}_4$ | Small, overlapping cleavable areas—Samples, medium size, thickness—(.02 mm.). |
| 15 | 67% $\text{KAlF}_4$<br>30% $\text{RbAlF}_4$<br>3% $\text{KBF}_4$ | Easily cleavable, large area, thin samples.                                   |
|    | 57% $\text{KAlF}_4$<br>40% $\text{RbAlF}_4$<br>3% $\text{KBF}_4$ | Easily cleavable, areas slightly smaller than above samples—samples thin.     |

20 The samples of the solid solution of potassium and rubidium fluoaluminates used in the above evaluations were single crystals as obtained from the melts. However, it is also possible to hot press small pieces of the fluoaluminate composition as is done with synthetic mica according to the process of U.S. 2,675,853.

25 It will be understood that capacitors may be made by techniques other than painting on or vacuum plating metal electrodes. For example, metal foils of aluminum, copper, and other electrically conducting materials may be used as the electrodes which are separated by the dielectric spacer. The fluoaluminate compositions are employed as is mica in conventional manufacturing techniques and U.S. Patents 1,345,754; 1,952,580; and 2,522,713 are illustrative of methods which may be used to make capacitors containing the fluoaluminate dielectric.

30 In addition to using the novel fluoaluminate compositions of this invention in a capacitor as demonstrated above, they may be used in other electric and electronic applications. For example, they may be used as electrode supports in vacuum tubes, in automated electronic manufactured articles employing wafer dielectrics for micromodule systems, in motor armature insulation, in high-voltage generator insulation in the form of tape fabricated from flakes of the fluoaluminate bonded to a backing, as dielectric insulators in switches, microswitches, relays, transformers, wires, and cables, coaxial cables, and the like, and in many electrical applications where dielectrics are generally used. In addition, they may be employed in place of glass as a binder for natural and synthetic mica used in pressed dielectrics. In this application they will have the advantage of supplementing the dielectric properties of the mica rather than adversely affecting the dielectric properties of the mica as does glass.

35 55 Many changes will be obvious to the skilled artisan and may be made from the above description of the invention without departing from its spirit and scope.

We claim:

1. Articles of manufacture containing an electrical conductor insulated with a solid dielectric wherein said dielectric is a crystalline solid solution consisting of  $\text{KAlF}_4$ ,  $\text{RbAlF}_4$  and  $\text{KBF}_4$  wherein the amount of  $\text{RbAlF}_4$  is at least about 4 mole percent and the amount of  $\text{KBF}_4$  is at least about 1 mole percent.

2. Articles of manufacture as in claim 1 wherein the amount of  $\text{RbAlF}_4$  is about 4 to 50 mole percent and the amount of  $\text{KBF}_4$  is 2 to 5 mole percent.

3. An electric capacitor comprising a sealed container, a pair of metal electrodes and a solid spacer therebetween, said spacer comprising a crystalline solid ternary solution consisting of about 4 to 90 mole percent of  $\text{RbAlF}_4$ , 1 to 5 mole percent of  $\text{KBF}_4$  and the balance of said ternary solid solution being  $\text{KAlF}_4$ .

4. A solid solution of a ternary mixture consisting of 75 at least about 4 mole percent of  $\text{RbAlF}_4$ , 1 to 15 mole

percent of  $\text{KBF}_4$  and the balance of said solid solution being  $\text{KAIF}_4$ .

5. A crystalline solid solution of a ternary mixture consisting of about 4 to 50 mole percent of  $\text{RbAlF}_4$ , 2 to 5 mole percent of  $\text{KBF}_4$  and the balance of said solution being  $\text{KAIF}_4$ .

6. A process for preparing a crystalline solid solution of a ternary mixture consisting of  $\text{KAIF}_4$ ,  $\text{RbAlF}_4$  and

$\text{KBF}_4$  by cooling a melt containing 67 mole percent of  $\text{KAIF}_4$ , 30 mole percent of  $\text{RbAlF}_4$  and 3 mole percent of  $\text{KBF}_4$ .

References Cited in the file of this patent

UNITED STATES PATENTS

3,016,480 Mockrin ----- Jan. 9, 1962